

Dec. 15, 1970

C. G. BIEBER ET AL.

3,547,625

STEEL CONTAINING CHROMIUM MOLYBDENUM AND NICKEL

Filed July 27, 1967



INVENTORS.  
CLARENCE G. BIEBER  
ROGER A. COVERT  
BY

M. L. Pisel  
ATTORNEY

**1**

3,547,625

**STEEL CONTAINING CHROMIUM MOLYBDENUM AND NICKEL**

Clarence George Bieber, Suffern, N.Y., and Roger Allen Covert, Middletown, N.J., assignors to The International Nickel Company, Inc., New York, N.Y., a corporation of Delaware  
Continuation-in-part of application Ser. No. 574,995, Aug. 25, 1966. This application July 27, 1967, Ser. No. 656,542

Int. Cl. C22c 39/20

U.S. Cl. 75—128

11 Claims

**ABSTRACT OF THE DISCLOSURE**

Iron-base alloys containing, among other constituents, interrelated amounts of nickel, molybdenum, and chromium offer a relatively high degree of resistance to various forms of corrosion in either or both the annealed and cold worked conditions. Alloys are also hot and cold workable and exhibit high tensile strength.

This is a continuation-in-part of application Ser. No. 574,995 filed Aug. 25, 1966.

The present invention relates to corrosion resistant alloys, particularly to iron-nickel alloys of novel composition and which are of comparatively low cost, both hot and cold workable, and which manifest enhanced resistance to corrosion, including crevice, pitting, intergranular and stress corrosion cracking, especially in chloride media, notably marine environments such as sea water.

As is generally well known, there has been a substantial increase over the years in the tonnage of metals and alloys used in resisting the corrosive effects of chlorides, including salt solutions, strongly oxidizing chloride solutions and marine environments. Commercial interest has been particularly expanding in respect of marine applications and this has been undoubtedly spurred by recent activities in offshore drilling, desalination, undersea mining, etc. However, unless improved and more corrosion resistant materials are developed, the heavy toll in metal damage inflicted by corrosion will continue to increase. It is perhaps interesting to reflect that a recent report indicates the overall loss exacted by corrosion is currently on the order of about five billion dollars annually. Such an economic burden self-explains the necessity of at least curtailing this trend.

A number of metals and alloys are currently being used or have been proposed for marine application, including the austenitic stainless steels, carbon and alloy steels, copper and copper alloys including various brasses, nickel alloys, titanium and alloys thereof, etc. However, depending upon intended purpose, such materials suffer from one or more drawbacks. The austenitic stainless steels, e.g., AISI 304, 310, 316, are readily workable and of reasonably low cost but do not exhibit superior resistance to crevice corrosion. This applies to an even greater extent concerning the carbon and low alloy steels. Copper alloys manifest a propensity to pit when immersed in stagnant sea water or when the rate of flow is less than about five feet per second (also true of austenitic stainless steels). This is not an unusual occurrence since it is known that as sea water velocity increases, fouling and pitting diminish in respect of many (although not all) materials. Certain nickel-base alloys have been used rather extensively. One of the most popular of such alloys contains about 17% chromium, 16% molybdenum and 4% tungsten but is costly and, at best, difficultly workable and usually requires several intermediate annealing treatments during the working cycle, a factor contributing to increased cost. Titanium and titanium alloys suffer from

**2**

the shortcoming of being of comparatively high cost and catastrophic corrosion has been experienced with certain titanium alloys.

The general problem is somewhat complicated by the fact that while certain applications require alloys which must resist chloride attack in the annealed condition, for other applications, e.g., marine cable (rope), it is more important that alloys manifest both high strength and exceptional resistance to chloride corrosives in the cold rolled condition. The ultimate, of course, would be to have available low cost alloys highly satisfactory in either condition, thus obviating concern as to which condition an alloy behaves more favorably. Each of these objectives is accomplished in accordance with the instant invention

which is addressed to the specific problem of providing low cost, hot and cold workable alloys which exhibit markedly improved resistance to crevice, pitting, intergranular and stress corrosion cracking in oxidizing chloride media, marine environments, etc.

It has now been discovered that the objectives above-discussed can be readily achieved with certain alloys containing special and correlated amounts of iron, nickel, chromium, molybdenum, and controlled amounts of aluminum, titanium, calcium, carbon, silicon, manganese, etc.

It is an object of the invention to provide improved iron-nickel-chromium-molybdenum alloys of novel composition.

Another object of the invention is to provide novel iron-nickel-chromium-molybdenum alloys of enhanced resistance to corrosive media, particularly chloride environments such as marine atmospheres, sea water, salt solutions, strongly oxidizing chloride solutions, etc.

It is a further object of the invention to provide new low cost, hot and cold workable corrosion resistant alloys.

Other objects and advantages will become apparent from the following description taken in conjunction with the accompanying drawing in which there is depicted a chart in respect of nickel and molybdenum contents pertaining to alloys within the invention as herein more fully described.

Generally speaking and in accordance with the present invention, alloys contemplated herein contain (in percent by weight) about 20% to 40% nickel, about 6% to 12% molybdenum, about 14% to 21% chromium, the chromium content being at least about 18% and advantageously at least 18.5% when the molybdenum content is not greater than about 6.5% or 7% and not exceeding 20% and preferably not exceeding 19% when the molybdenum content is from 10% to 12%, up to 0.2% carbon, up to 0.5% silicon, up to 1% but beneficially not more than 0.5% manganese, the sum of the silicon plus manganese not exceeding about 1.25%, up to 0.7% titanium, up to 0.7% aluminum, up to about 0.15% calcium, up to 12% cobalt, and the balance essentially iron, the iron constituting at least 30% of the alloys. In consistently achieving good hot workability characteristics, the alloys advantageously contain titanium or aluminum (most beneficially both) in amounts of from 0.05% to 0.6% each, e.g., 0.15% to 0.5%. Further, it is most preferred and desirable that the alloys contain calcium, e.g., 0.001% or 0.01% to 0.15% calcium, in consistently achieving highly satisfactory results. The theory which might explain the role of calcium is not completely understood, but apart from other possible benefits, it has been found that calcium markedly influences and enhances resistance to crevice corrosion in both the annealed and cold worked conditions, particularly the latter and particularly with regard to alloys containing not more than about 8% molybdenum, e.g., 7.5% molybdenum, or lower. Calcium must be present when the molybdenum content of the alloys

is not greater than about 7.5% or 8%; otherwise, crevice corrosion resistance is adversely affected even in the annealed condition.

Other constituents which can be present in the alloys include the following: up to 2%, e.g., up to 0.5% or 1%, columbium, up to 1% vanadium, up to 1% copper, up to 1% tungsten and up to 2% tantalum. However, elements such as phosphorus, sulfur, oxygen, nitrogen, and the like should be kept at low levels consistent with good commercial practice. Sulfur is deemed particularly detrimental and particular care should be exercised in this regard. It is thought that one of the attributes of calcium is that it counteracts the deleterious effects of sulfur. Nitrogen should be maintained below about 0.03%, preferably below about 0.01%.

In carrying the invention into practice, the alloys should contain at least 20% nickel. With nickel levels lower by an appreciable extent, corrosion resistance in marine and other environments is not only unsatisfactory but there is the added danger of forming delta ferrite. If present in an excessive although relatively low amount, delta ferrite promotes or potently contributes to embrittlement problems whereby workability is, at best, impaired. In this connection and in accordance with the invention, the alloys should be substantially austenitic (single phase) and devoid of detrimental delta ferrite and/or other deleterious phases such as sigma.

Further, consistently highly satisfactory results do not always obtain even with nickel contents of, say, about 20% to 23%. For example, when the content of molybdenum in the alloys is above about 9.5%, e.g., 10%, and up to 12%, it has been found that unless the nickel content exceeds about 23%, both hot and cold workability are rendered more difficult such that intermediate annealing may be required and this increases cost. Moreover, at a nickel level of less than about 23%, resistance to crevice corrosion, especially in respect of alloys in the cold rolled condition, is inferior when both the molybdenum and chromium are at the low end of their respective ranges. When the nickel content is as low as 20% and the molybdenum content is from 6% to about 6.5%, the alloys should contain about 18% or more of chromium, e.g., 18.5%, as indicated above herein. Generally speaking, at a molybdenum level above about 6.5% to about 7.5%, a chromium content of about 17% and upwards should be used with nickel contents as low as 20%. At about 7.5% to 8% molybdenum, about 15.5% or 16% chromium and above can be used with such low (as well as higher) nickel contents. It is beneficial, however, for an optimum combination of resistance to crevice corrosion coupled with good workability, that the alloys contain at least 23% and more advantageously at least 24% or 25% nickel.

In respect of the higher end of the nickel range, to wit, 35% to 40% nickel, a particularly noteworthy feature of the invention stems from the fact that not only is resistance to crevice and pitting corrosion and the like markedly good in chloride media but resistance to stress corrosion cracking is excellent. As will be illustrated herein, this obtains not only in marine environments, sea water, but most significantly when the alloys are exposed to the extreme aggressive attack so characteristic of boiling magnesium chloride. Alloys resistant to stress corrosion cracking should contain, in addition to 35% to 40% nickel, above about 9%, e.g., 9.5%, and up to 12% molybdenum and about 14% to not more than about 19% chromium, the balance of the composition being in accordance with that given before herein. Up to 10% cobalt can be used to replace an equivalent amount of nickel. Where outstanding resistance to crevice and pitting corrosion coupled with resistance to stress corrosion cracking is required, it is beneficial that the alloys contain, in addition to a nickel plus cobalt content of about 35% to 40%, about 10% to 12% molybdenum and about 14% or 15% to 18% chromium.

Low molybdenum contents result in inferior resistance to crevice corrosion. For example, molybdenum contents of 4% are markedly poor. Too, as will be shown herein, an amount of molybdenum of, say, 6% is quite unacceptable should the chromium content be on the low side, e.g., 14% to 17%. It is most advantageous that at least 8% molybdenum be present in the alloys and even then satisfactory results will not consistently obtain unless the molybdenum, nickel, and also the chromium contents are correlated. In this regard, it is not a question of using high nickel contents to attain a desired degree of resistance. Increasing the amount of nickel beyond about 27% or 28% has been found to result in lower crevice corrosion resistance at molybdenum levels of about 7%. But by using 8% or more of molybdenum particularly with chromium contents of at least 17%, highly satisfactory results can be obtained at higher nickel levels. The correlation between nickel and molybdenum is represented by the accompanying drawing. It should be pointed out that with respect to the area, ABCLA, an area encompassing a fair number of alloys at nickel percentages above 28% but amounts of molybdenum of less than 8%, the chromium content for such compositions should be about 18% or more.

In addition and subject to the foregoing, where resistance to stress corrosion cracking in potently aggressive agents such as boiling magnesium chloride is not necessary, and thus a nickel minimum of 35% is not required, highly satisfactory results are attained when the molybdenum and nickel contents are interrelated to represent a point within the area ABCDEFA of the accompanying drawing, the chromium content of the alloys advantageously being from 14% or 15% to 20%, e.g. 17% to 20%. Alloys containing from about 15% to 20% chromium and having molybdenum and nickel contents representing a point falling within the area BGHJKB, and particularly within the area GHJKG, are deemed especially attractive commercially since they would be the most economical, are readily amenable to both hot and cold working, and provide good resistance to crevice corrosion in both the hot and cold worked conditions.

In addition to what has been said before herein in respect of chromium and while it contributes to resisting corrosive attack, excessive amounts thereof can lead to poor results, particularly by promoting a multiple phase structure. This, in turn, would bring about adverse consequences. A chromium content of, say, 22%, part from being unnecessary, is particularly undesirable to molybdenum levels of 9% and above. Accordingly, when the molybdenum content is from about 9.5% or 10% to 12%, the chromium content, as indicated before herein, should not exceed 20% and advantageously does not exceed about 19%.

Careful control must be exercised with regard to silicon and manganese. Silicon in appreciable quantities, e.g., 1% or 2%, is notably undesirable by reason of the fact that it impairs hot workability and weldability. Manganese in comparatively high amounts, e.g., 1.5% to 2%, also significantly impairs corrosion resistance. As indicated above herein, it is preferred that the total silicon plus manganese content not exceed 1.25%. Advantageously, the silicon content should not exceed 0.25% and the total silicon plus manganese should not exceed about 0.75%.

Although the amount of carbon in the alloys can be as high as 0.2%, carbon somewhat in excess of 0.1%, e.g., 0.15%, results in diminishing crevice corrosion resistance in otherwise outstanding alloys. In achieving both good crevice corrosion resistance and resistance to intergranular corrosion, it is advantageous that the carbon content not exceed about 0.05%, e.g., 0.03%, or less. However, in this regard, columbium when present, will combine with the carbon such that carbon contents up to 0.1% are satisfactory. Columbium also obviates the necessity of solution treating weldments.

Particularly satisfactory hot workability characteristics are conferred by titanium and/or aluminum. Contributing

to the desideratum of low cost is the fact that air melting techniques can be employed. Thus recourse to more expensive processing is unnecessary. Titanium is also useful to stabilize nitrides, thereby preventing the occurrence of porosity in ingots. Accordingly, it is preferred that at least one, beneficially both, of these constituents be present in amounts of at least 0.05%, advantageously at least 0.1% or 0.25%, and up to 0.5%. Appreciable amounts of these elements, however, e.g., 1.5% or 2%, are quite undesirable since the net effect would be to subvert working characteristics without benefit corrosionwise.

As indicated herein, air melting practice can be readily employed in preparation of the alloys, although vacuum techniques can also be used. It might be mentioned, as will be appreciated by those skilled in the art, recovery of titanium and/or aluminum and/or calcium is usually not 100%. Where it is desired that the alloys contain about 0.15% of titanium or aluminum, about 0.25% of each should be added to the melt. Calcium, which can be incorporated in the form of a calcium-silicon addition,

tested in the cold rolled and also in the annealed condition. Cold rolled specimens having a surface area of about 25 square centimeters were immersed for about 72 hours in the 10% ferric chloride solution, rubber bands being wrapped thereabout to intentionally create crevices. This test is deemed equivalent to an extreme long-time exposure in sea water and is described by M. A. Streicher in Journal of the Electrochemical Society, vol. 103, pages 375-390, No. 7, July 1956. Other cold rolled specimens of the same alloys (same area) were annealed at about 2150° F. to 2200° F. for about one-half hour and tested in the annealed condition and in the same manner as the cold rolled specimens. Nominal compositions and data are given in Table I for both the cold rolled and the annealed specimens. In addition to the percentages of the various constituents set forth in Table I, about 0.03% carbon (except Alloy 21), 0.1% silicon, 0.15% manganese, and about 0.06% calcium (as calcium-silicon) were added to the melts. Both titanium and aluminum were used in preparing the alloys, about 0.25% of each being added.

TABLE I

| Alloy: | Ni, percent | Cr, percent | Mo, percent | Other, percent | Fe, percent | Weight loss in milligrams |              |
|--------|-------------|-------------|-------------|----------------|-------------|---------------------------|--------------|
|        |             |             |             |                |             | Cold rolled               | and annealed |
| 1      | 23          | 17          | 8           | Balance        | 3.5         | 2.4                       |              |
| 2      | 25          | 17          | 8           | do             | 4.8         | 1.6                       |              |
| 3      | 25          | 17          | 8           | do             | 0.9         | 0.8                       |              |
| 4      | 25          | 17          | 8 0.5 Cb    | do             | 1.8         | 2.1                       |              |
| 5      | 25          | 20          | 8           | do             | nil         | 0.4                       |              |
| 6      | 27          | 20          | 8           | do             | 0.9         | 0.4                       |              |
| 7      | 25          | 14          | 10          | do             | 1.1         | 3.3                       |              |
| 8      | 28          | 14          | 10          | do             | 0.8         | 0.6                       |              |
| 9      | 30          | 14          | 10          | do             | 0.6         | 1.0                       |              |
| 10     | 27          | 15          | 10 0.5 Cb   | do             | 1.1         | 1.3                       |              |
| 11     | 35          | 15          | 10 0.5 Cb   | do             | 2.5         | 1.6                       |              |
| 12     | 40          | 15          | 10 0.5 Cb   | do             | 3.5         | 2.1                       |              |
| 13     | 25          | 17          | 10          | do             | 1.1         | 0.4                       |              |
| 14     | 28          | 17          | 10          | do             | 2.1         | 1.2                       |              |
| 15     | 30          | 17          | 10          | do             | 1.8         | 2.7                       |              |
| 16     | 27          | 18          | 10 10 Co    | do             | 0.3         | 0.3                       |              |
| 17     | 35          | 15          | 12 0.5 Cb   | do             | 9.1         | 7.5                       |              |
| 18     | 40          | 15          | 12 0.5 Cb   | do             | 2.2         | 4.1                       |              |
| 19     | 27          | 18          | 12          | do             | 0.5         | 0.4                       |              |
| 20     | 30          | 18          | 12          | do             | 0.7         | 0.3                       |              |
| 21     | 25          | 17          | 8 0.15 C    | do             | 17.5        | 10.8                      |              |
| 22     | 20          | 14          | 10          | do             | 2.9         | 2.6                       |              |
| 23     | 23          | 14          | 10          | do             | 5.1         | 6.4                       |              |
| 24     | 20          | 17          | 10          | do             | 1.3         | 2.6                       |              |
| 25     | 23          | 17          | 10          | do             | 5.0         | 5.3                       |              |

should be added in an amount of about two to three times that desired in the final alloys. Ingots can be hot worked from about 2200° F. to 2300° F. down to about 1800° F. to 1600° F. Suitable annealing temperatures include about 2000° F. to 2300° F., e.g., 2200° F. A final annealing temperature of about 2200° F. has been found satisfactory. In producing strip and the like, the alloys can be hot rolled, annealed, pickled and cold rolled. Intermediate annealing between cold rolling stages can be carried out over the temperature range of 2000° F. to 2200° F. It is rather ironic to note that it has been found difficult to pickle the alloys due to the exceptional corrosion resistance thereof.

In order to give those skilled in the art a better appreciation of the invention, the following illustrative description and data are given:

A substantial number of alloys (Alloys 1 through 25, Table I) within the invention were prepared using air melting techniques. Ingots were soaked at about 2300° F. and thereafter hot rolled to billets, the hot working temperature range being on the order of 1600° F. to 2300° F.

The hot rolled alloys were annealed at about 2150° F. to 2200° F. for about one-half hour and were cold rolled to strip about  $\frac{1}{16}$  inch thick (the hot rolled thickness was approximately  $\frac{1}{4}$  inch). Corrosion tests were conducted using an aggressive corrodent commonly used for test purposes, to wit, a 10% ferric chloride solution. In this regard, two different tests were conducted. Specimens were

50 In respect of the data in Table I, it is clear that Alloys 1 through 20 exhibited highly satisfactory resistance to crevice corrosion. No pitting was observed. Regarding Alloy 21, this alloy nominally contained 0.15% carbon, the composition otherwise being the same as for Alloys 2 and 3. While Alloy 21 is acceptable for castings and for applications concerning alloys in the annealed condition, 55 it will be noted that the high carbon content resulted, comparatively speaking, in quite a loss in crevice corrosion. As indicated above herein, it is much more desirable to maintain the carbon content at a level not above 0.1% and advantageously less than 0.05% or 0.03%. (It should be mentioned that alloys to be acceptable in the 10% ferric chloride test described herein should not manifest a loss greater than about 15 milligrams and advantageously not greater than about 10 milligrams, the optimum being a maximum loss of about 5 milligrams.)

60 Some difficulty was experienced in hot working Alloys 22 through 25, particularly Alloys 22 and 24 (which alloys contained only 20% nickel), although crevice corrosion resistance was good. Edge cracking was noted primarily in respect of Alloys 22 and 24 and with such low nickel contents, in combination with the molybdenum content of 10%, intermediate annealing would be necessary. However, as referred to herein and as illustrated by Alloys 7 and 13, nickel contents above 23%, to wit, 25%, resulted in good hot working characteristics.

65 Both cold rolled and annealed specimens of Alloys 3,

10, 11, 16 and 17 were exposed to sea water at ambient temperature (flow of 2 feet per second) at the renowned testing station at Harbor Island, N.C. Specimens to determine both crevice corrosion and stress corrosion cracking (U-bends) behavior were employed. Alloy 3 was exposed for a period of about 450 days, each of the others being exposed for about 300 days (exposure continues in all cases), examinations being made periodically. Each of the specimens was free of any evidence of stress corrosion cracking. A very slight and inconsequential amount of crevice corrosion was observed in connection with the cold rolled specimen of Alloy 3 after 90 days, but this proved to be very incipient and did not progress further. It is more than likely that machining prior to exposure was not perfect. In summary, the specimens behaved remarkably well.

U-bend specimens of Alloys 2, 3, 10, 11, 12 and 16 were also exposed to boiling 42% magnesium chloride (154° C.) to determine stress corrosion cracking tendencies under the extremely severe conditions imposed by this test (a test commonly used to determine stress corrosion cracking behavior of the austenitic stainless steels).

5  
10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955  
8960  
8965  
8970  
8975  
8980  
8985  
8990  
8995  
9000  
9005  
9010  
9015  
9020  
9025  
9030  
9035  
9040  
9045  
9050  
9055  
9060  
9065  
9070  
9075  
9080  
9085  
9090  
9095  
9100  
9105  
9110  
9115  
9120  
9125  
9130  
9135  
9140  
9145  
9150  
9155  
9160  
9165  
9170  
9175  
9180  
9185  
9190  
9195  
9200  
9205  
9210  
9215  
9220  
9225  
9230  
9235  
9240  
9245  
9250  
9255  
9260  
9265  
9270  
9275  
9280  
9285  
9290  
9295  
9300  
9305  
9310  
9315  
9320<br

was characterized by such poor hot workability that corrosion tests in the cold rolled and annealed conditions were not made. It will be noted the alloy contained high silicon (1.1%) and titanium (2%) contents as well as a high amount of silicon plus manganese (1.8%). In most marked contrast thereto are Alloys 15 and 9, alloys within the invention.

As indicated above herein, neither calcium nor titanium or aluminum was added to the melts of Alloys HH through PP and 27, 28 and 29. In this regard, JJ through MM, 27, 28 and 29 (also Alloy 5) are of particular interest. As will be observed, Alloys JJ, KK and LL each exhibited poor corrosion resistance whether in the cold rolled or annealed condition. Alloys 27, 28 and 29, however, were satisfactory in the annealed condition and are thus within the invention for that reason. It is, of course, interesting to compare Alloy 5 (which contained calcium and also titanium and aluminum) with Alloys 27, 28 and 29. It is thought the difference in results is strikingly remarkable.

Alloys 30 through 39, 3 and QQ illustrate in a general manner alloy behavior as the nickel content is increased over the lower end of the molybdenum range. Note that Alloy 32 is an extremely marginal composition at best and only then in the annealed condition. With 18% chromium, an otherwise similar alloy (Alloy 31) exhibited considerably better corrosion resistance whereas, increasing the nickel content to 30% as in Alloy QQ resulted in inferior resistance particularly in the cold rolled condition. As indicated before herein, improper correlation of the nickel and molybdenum contents can lead to poor results. Alloys 3, 35 and 34 afford an interesting comparison with Alloy 39 concerning the effect of increasing the chromium content (16.6% to 21%) as the percentage of nickel increased (25% to 34%). The standard stainless steels AISI 310 and 316 as well as prior art Alloys NN and PP behaved poorly in test.

Alloys contemplated within the invention are generally useful for vessels, boat hulls, and structures and components therefor employed in (or in the vicinity of) marine environments, including sea water and sea atmospheres. More specifically, the alloys are useful for pumps and parts therefor (including vanes and impellers), propellers, pipes, valves, fasteners, tubing in general including heat exchanger tubing and tube sheet, water boxes, seawater evaporators, including plate, shafting, marine hardware, e.g., chocks, cleats, pulleys, wrought fittings, trim and fasteners, buoys, floating platforms, oil well equipment, etc. Chemical plant equipment for handling of oxidizing acids and salts thereof, containers and pressure vessels for the storage or transportation of various corrosive chemicals are illustrative of other uses for the alloys. Also, the alloys can be used in conventional mill forms including sheet, strip, bar, rod, etc.

Although the present invention has been described in conjunction with preferred embodiments, it is to be understood that modifications and variations may be resorted to without departing from the spirit and scope of the invention, as those skilled in the art will readily understand. Under certain circumstances it may be permissible to use magnesium together with or in place of calcium but it is much preferred to use the latter. Such modifications and variations are considered to be within the purview and scope of the invention and appended claims.

We claim:

1. An iron-nickel-molybdenum-chromium alloy characterized by enhanced resistance to various corrosive chloride environments, said alloy consisting essentially of about 20% to 40% nickel, about 6% to 12% molybdenum, the nickel and molybdenum being correlated to represent a point falling within the area LFEDCL of the accompanying drawing, about 14% to 21% chromium, the chromium being (a) at least about 18% when the molybdenum content is not greater than about 6.5% and (b) not greater than 20% when the molybdenum content is from about 10% to 12%, up to 0.05% carbon,

up to 0.15% calcium with the proviso that at least 0.001% of calcium is present when the molybdenum content is not greater than about 7.5%, at least one metal selected from the group consisting of titanium in an amount up to about 0.7% and aluminum in an amount up to about 0.7%, up to about 12% cobalt, up to 0.5% silicon, up to 1% manganese, the sum of any silicon and manganese not exceeding 1.25%, up to 1% columbium, up to 1% vanadium, up to 1% copper, up to 1% tungsten, up to 2% tantalum and the balance essentially iron.

2. An alloy as set forth in claim 1 containing at least 23% nickel and in which columbium, if present, does not exceed about 0.5%.

3. An alloy as set forth in claim 1 and containing about 0.001% to 0.15% calcium and from 6.5% to 8% molybdenum.

4. An iron-nickel-molybdenum-chromium alloy characterized by enhanced resistance to various corrosive chloride environments, said alloy consisting essentially of about 20% to 40% nickel, about 6% to 12% molybdenum, the nickel and molybdenum being correlated to represent a point falling within the area ABCDEFA of the accompanying drawing, about 14% to 21% chromium, the chromium being (a) at least about 18% when the molybdenum content is not greater than about 6.5% and (b) not greater than 20% when the molybdenum content is from about 10% to 12%, up to 0.05% carbon, up to 0.15% calcium with the proviso that at least 0.001% of calcium is present when the molybdenum content is not greater than about 7.5%, at least one metal selected from the group consisting of titanium in an amount up to about 0.7% and aluminum in an amount up to about 0.7%, up to about 12% cobalt, up to 0.5% silicon, up to 1% manganese, the sum of any silicon and manganese not exceeding 1.25%, up to 1% columbium, up to 1% vanadium, up to 1% copper, up to 1% tungsten, up to 2% tantalum and the balance essentially iron.

5. An alloy as set forth in claim 4 wherein calcium is present in an amount of at least 0.001%.

6. An alloy as set forth in claim 4 and containing at least one metal from the group consisting of titanium and aluminum in an amount of 0.05% to 0.6% of each.

7. An alloy as set forth in claim 4 in which silicon does not exceed 0.25% and manganese does not exceed 0.5%.

8. An iron-nickel-molybdenum-chromium alloy consisting essentially of from 23% to 30% nickel, from about 8% to about 10% molybdenum, the nickel and molybdenum being correlated to represent a point within the area BGHJKB of the accompanying drawing, about 15% to about 20% chromium, up to 0.05% carbon, up to 0.15% calcium, at least one metal selected from the group consisting of titanium in an amount up to 0.7% and aluminum in an amount up to 0.7%, up to 12% cobalt, up to 0.5% silicon, up to 1% manganese, the sum of the silicon plus manganese not exceeding 1.25%, up to 2% of columbium, up to 1% of vanadium, up to 1% copper, up to 1% tungsten, up to 2% tantalum and the balance essentially iron.

9. An alloy as set forth in claim 8 in which calcium is present in an amount of at least 0.01%.

10. An alloy as set forth in claim 8 in which silicon does not exceed about 0.25% and manganese does not exceed about 0.5%.

11. An iron-nickel-molybdenum-chromium alloy which manifests excellent resistance to stress corrosion cracking and crevice corrosion in chloride media, said alloy consisting essentially of about 25% to 40% nickel, about 9.5% to 12% molybdenum, about 14% to 19% chromium, up to 0.05% carbon, up to 0.15% calcium, at least one metal selected from the group consisting of titanium in an amount up to 0.7% and aluminum in an amount up to 0.7%, up to 0.5% silicon, up to 1% manganese, the sum of the silicon plus manganese being not greater than about 1.25%, up to 12% cobalt, the sum of the cobalt

plus nickel being at least about 35%, up to 2% columbium, up to 1% vanadium, up to 1% copper, up to 1% tungsten, up to 2% tantalum and the balance essentially iron.

## References Cited

## UNITED STATES PATENTS

- 2,398,702 4/1946 Fleischmann ----- 75-128.9  
 2,403,128 7/1946 Scott ----- 75-171

|           |         |                |          |
|-----------|---------|----------------|----------|
| 2,570,193 | 10/1951 | Bieber -----   | 75-171C  |
| 2,809,127 | 10/1957 | Gibson -----   | 75-128.9 |
| 3,048,485 | 8/1962  | Bieber -----   | 75-171H  |
| 3,094,414 | 6/1963  | Franklin ----- | 75-171A  |
| 3,107,167 | 10/1963 | Abkowitz ----- | 75-171H  |
| 3,183,084 | 5/1965  | Heydt -----    | 75-128.9 |

HYLAND BIZOT, Primary Examiner